

Dec. 12, 1933.

G. A. RICHTER

1,938,722

RIPENING OF VISCOSE SIRUP

Filed Dec. 8, 1930



Inventor  
George A. Richter  
Kugler, Brown, Quincy & May  
Attys

## UNITED STATES PATENT OFFICE

1,938,722

## RIPENING OF VISCOSE SIRUP

George A. Richter, Berlin, N. H., assignor to  
Brown Company, Berlin, N. H., a corporation  
of Maine

Application December 8, 1930. Serial No. 500,689

4 Claims. (Cl. 260—100)

This invention relates to a process of ripening or maturing viscose sirup, more particularly from the standpoint of attaining that physical and chemical condition in the sirup at which it is ready and satisfactory for manufacture into products of the type of artificial silk filaments.

When cellulose xanthate is dissolved in caustic soda solution to form viscose sirup, so called, the fresh or unripened sirup cannot successfully be spun into the usual acid-setting baths, for the reason that cellulose is not regenerated from the xanthate to a sufficient extent and at the proper rate to give rise to filaments of the desired tenacity, strength, elasticity, and other characteristics. In order to realize these desiderata, it has been found necessary to subject the viscose sirup to what is known as a ripening operation, during which operation it is generally understood that combined sulphur splits off and the cellulose complex becomes progressively poorer in sulphur. The ripening is carried to a point short of gelling of the sirup, for were gelling to take place, it would be impossible to handle the gel in the usual spinning machines without serious gumming and plugging of the pipe lines, pumps, spinnerets, and other parts. The customary practice in producing satisfactorily spinnable viscose sirups is to form a cellulose xanthate solution in caustic soda containing 7% cellulose, calculated as cellulose but in the form of xanthate, and 6½% caustic soda. This sirup, which is of a thick consistency not unlike molasses, is then filtered to remove undissolved fibers and other solid impurities which would tend to interfere with spinning by plugging the orifices of the spinnerets. The filtered sirup is then delivered to a storage tank, wherein it is stored or allowed to ripen under controlled low temperature conditions, usually 20° C., until it acquires the composition requisite for successful spinning. Depending upon the nature of the fresh or unripened sirup, it usually takes from about 72 to 96 hours standing at 20° C. to produce a fully and satisfactorily ripened sirup.

There are many disadvantages inherent in a viscose-ripening procedure such as hereinbefore described. Thus, the equipment required is expensive and occupies much space, including, as it does, a special thermo-insulated room, an elaborate system of refrigeration, control of the atmosphere of the room, a large number of storage tanks for the viscose sirup, and pumps for circulating the sirup. Again, a large inventory or stock of sirup must always be on hand; and if the sirup is damaged or completely spoiled, a

delay of three to four days must be contended with before the inventory is adjusted to catch up with the requirements of the spinning machines, assuming that the plant is an efficient one equipped with the number of spinning machines 60 to consume the entire output of the ripening apparatus.

I have discovered that the time necessary for ripening viscose sirup may be reduced to a comparatively insignificant period, if the fresh or unripened sirup is heated to a temperature materially above normal room temperature. The particular temperature to which the sirup is heated and the time period to be allotted for heating depends on various factors, especially 70 upon the composition and characteristics of the sirup, which determine its tendency to split off combined sulphur and thereby to regenerate cellulose. In my application Serial No. 484,292, filed September 25, 1930, I have disclosed and 75 claimed the principles of my discovery, as well as one specific method and apparatus embodying these principles. I have now found that the desired results may be realized by depositing an unripened viscose sirup as a film on a smooth, 80 non-absorbent, heated surface, and keeping the sirup film in contact with the heated surface only for a sufficient time interval to effect the desired ripening, that is, without causing gelling to take place. I have further found that 85 the time interval for heating in such case need be so short that the sirup may be progressively deposited on a heated carrier moving circuitously at the appropriate rate of speed, and then be progressively removed in a ripened but ungelled 90 condition only an exceedingly short time after its deposition and before the carrier has completed a circuit. Such a process is advantageous, as it not only makes possible quick, high-capacity production of ripened viscose sirup, but 95 also lends itself to easy control to produce ripened sirup of the proper quality. Thus, such factors as the temperature of the surface on which the sirup is deposited may be controlled thermospatially when the surface is heated either by 100 steam, electrical units, or the like; and the station for removing the sirup film from the carrier may be shifted to ensure a removal when the sirup has reached the desired condition. A convenient and available type of carrier is a 105 steel drum whose periphery is nicely finished and which is heated internally by steam. When the drum is slowly revolved so that a portion of its periphery comes in contact with a supply of viscose sirup, a film of sirup forms over the 110

periphery of the drum, owing to the adhesive-  
ness and viscosity of the sirup. The sirup car-  
ried by the drum periphery may be readily re-  
moved as by a rubber or metal doctor blade.  
5 The use of a smooth, non-absorbent surface for  
receiving the viscose sirup makes possible the  
removal of practically all the sirup, but traces  
of residual sirup may be removed by sprays  
and/or brushes before the cleared surface again  
10 comes in contact with the supply of unripened  
sirup.

In order to make possible the keeping of the  
ripened sirup in ungelled condition for a sub-  
stantial period of time, it is cooled promptly  
15 after ripening, preferably in a manner similar  
to that of its heating, to temperatures down-  
wards of 20° C., as at such temperatures it may  
be allowed to stand as a batch for some hours,  
without danger of gelling. In other words, the  
20 hot, ripened sirup may be cooled by the use  
of apparatus similar to that employed in its  
heating, except that the drum periphery on  
which it is deposited is cooled, rather than being  
heated.

25 With the foregoing and other features and ob-  
jects in view, my invention will now be further  
described in conjunction with the accompany-  
ing drawing, wherein

Figures 1 and 2 show diagrammatically and  
30 conventionally different forms of apparatus in-  
volving the use of both heating and cooling  
drums.

Figures 3 and 4 represent sections through a  
heating and cooling drum, respectively.

35 In Figure 1, I have shown a vat 1, in which  
is maintained a bath of unripened viscose sirup.  
The sirup may be continuously delivered into  
the bath from a suitable source of supply,  
through a pipe 2, at a rate corresponding to  
40 the rate of removal of sirup from the bath.  
Rotating partially submerged in the bath of  
sirup is a steam-heated drum 3, which continu-  
ously picks up a film of sirup and carries it  
out of the bath. As shown in Figure 3, the  
45 ends of the drum have trunnions 4, in which are  
fitted glands 5. Through one of these glands  
a steam-supply pipe 6 passes upwardly into the  
hollow of the drum. Through the other of these  
50 glands, a steam outlet pipe 7 enters into the  
hollow of the drum, this latter pipe preferably  
terminating as a T having an upwardly ex-  
tending portion 8 to carry out the steam, and  
a downwardly extending portion 9 to carry out  
55 the condensate. Uniformity of the film of sirup  
clinging to the periphery of the drum may be  
ensured by a roll 10 arranged somewhat above  
the surface of the bath and rotating in contact  
with the film in a direction opposite to the ro-  
60 tational direction of the drum. The roll 10 is  
preferably adjustable to vary the clearance be-  
tween it and the drum, and thus to determine  
the thickness of the film remaining on the drum.  
The film of sirup is carried by the drum pe-  
65 riphery for a while, but immediately before the  
line of dipping into the bath it is scraped from  
the drum periphery by a doctor blade 11, which  
also serves to direct the ripened sirup into a  
second vat 12. The bath of hot, ripened sirup  
70 thus formed in the bath 12 is cooled by em-  
ploying instrumentalities similar to those used  
in heating the unripened sirup delivered into  
the vat 1. That is to say, I use a drum 13,  
a distributing roll 14, and a doctor blade 15,  
75 but the periphery of the drum 13 is cooled,  
rather than being heated. The cooling drum 13,

as shown in Figure 4, may be of a construc-  
tion similar to the heating drum 3. When a  
liquid cooling medium such as chilled brine is  
circulated through the cooling drum, it is pref-  
erable that the brine be fed downwardly into  
80 the drum hollow from a supply pipe 16, and  
that a discharge pipe 17 project upwardly into  
the drum hollow, as in such case the warmest  
brine tends to rise to the top of the pool of  
brine maintained in the drum and flow into the  
85 discharge pipe. The cooled sirup removed from  
the drum 13 may be directed by the doctor blade  
15 into a tank 18, from which it may be with-  
drawn for use as desired.

The apparatus shown in Figure 2 is similar  
to that shown in Figure 1, except that the vats  
have been dispensed with and in their stead I  
have made provision to maintain banks of sirup  
in contact with the drums. To this end, I have  
arranged a heating drum 19 at a level above  
90 that of a cooling drum 20, each of said drums  
rotating in contact with the lower edge of an  
inclined platform or shelf 21 having end-pieces  
(not shown) and which serves to form, with  
one side of the drum, a reservoir for holding  
100 a bank of sirup. As the heated drum rotates,  
it picks up a film of sirup from the bank con-  
stantly maintained on the upper platform, and  
carries it to the other side, where it is removed  
by a doctor blade 22 onto the lower platform.  
105 Such an apparatus has the advantage that con-  
siderable periphery surface of the drum is ex-  
posed for the action of cleaning means, such  
as brushes 23, between the doctor blade and  
the station for supplying the viscose sirup.  
110

While the temperature of the periphery of the  
heating drum may be varied from, say, 50°  
115 to 120° C., nevertheless, even taking into con-  
sideration the wide variabilities possible in the  
nature of unripened viscose sirups, the operat-  
ing temperature range need not fall outside of  
120 between 60° to 100° C. The particular tempera-  
ture employed depends, among other factors,  
upon the alkali content of the sirup when it is  
prepared. The usual sirup contains 7% cellulose  
125 and 6½% caustic soda, but for some purposes  
one might prefer a sirup containing the same  
amount of cellulose, but a materially lower  
amount of alkali, say, 3% to 3½% caustic soda.  
Sirups of such reduced caustic soda content are  
130 ripened very quickly at temperatures not above  
70° to 75° C. If desired, the sirup may be  
warmed somewhat, or partially ripened, before  
it is brought into contact with the heating drum,  
but when using a sirup which is thin or of low  
135 viscosity, it may be of advantage to increase its  
viscosity by cooling it somewhat, in order to  
enhance its adhesiveness to and distribution  
over the heating drum. The heating treatment  
of the sirup may be carried out in an atmos-  
phere of sufficient humidity to avoid much  
140 evaporation of water therefrom, as evaporation  
of considerable water is conducive to gelling.  
The use of a humid atmosphere may be es-  
pecially desirable if the heat treatment is car-  
ried out at temperatures above 90° C., at which  
145 there would be considerable tendency for the  
evaporation of water from a film of sirup unless  
such evaporation were inhibited by a suitably  
humid atmosphere. The heat-ripened sirup  
may be kept hot for a while, although, as al-  
ready indicated, it is usually desirable to effect  
its cooling promptly to temperatures downwards  
of 20° C., unless the ripened sirup is to serve  
150 immediately for the manufacture of artificial

- silk filaments or the like. In fact, it may be desirable to cool the heat-ripened sirup to as low as 10° C., at which temperature it may be preserved for days without appreciable change, whereas a batch of ripened sirup at 22° C. must be spun within about five to six hours, in order to avoid non-uniformity of the artificial silk spun therefrom, by reason of the fact that the last portions of the batch are liable to undergo spontaneous variation from the first portions of the same batch. When the sirup is of unusually high viscosity, so that it may be spun only with difficulty at temperatures downwards of 20° C., it is advantageous to spin the heat-ripened sirup in a hot condition immediately as it is produced, as the hot sirup is of low viscosity and so lends itself to good spinning. The normal sirups, however, even when at temperatures as low as 10° C., not only spin satisfactorily, but generally yield a better quality of silk at low temperatures, because regeneration of cellulose is accompanied by less violent liberation of hydrogen sulphide, which at high temperatures tends to occlude to the nascent silk filaments and to break them. If desired, however, the heat-ripened sirup may initially be chilled to the desired temperature whereat it may be kept stable, and the cold sirup then heated to the desired temperature and viscosity immediately before spinning.
- The embodiment of my invention hereinbefore described may further be varied while still falling within the ambit of the invention. For instance, rather than carrying out a one-stage heating of the sirup, the heating step may be performed in stages by using a series of two or more heating drums, the temperature imparted to each drum in the series being different from
- and controlled independently of the temperatures of the other drums.
- I claim:
1. A process which comprises progressively depositing an unripened viscose sirup as a film on a heated surface under atmospheric pressure; and progressively removing the heated film of sirup from such heated surface in a ripened but ungelled condition. 80
  2. A process which comprises progressively depositing an unripened viscose sirup as a film on a heated surface under atmospheric pressure, progressively removing the heated film of sirup from such heated surface in a ripened but ungelled condition; progressively depositing the hot, ripened but ungelled sirup on a cooled surface; and progressively removing the cooled film of ungelled sirup from such cooled surface. 85 90
  3. A process which comprises depositing an unripened viscose sirup as a film on a heated surface under atmospheric pressure and enveloped in a humidified atmosphere serving to inhibit the evaporation of water from said sirup; and removing the heated film of sirup from such heated surface in a ripened but ungelled condition. 95 100
  4. A process which comprises progressively depositing an unripened viscose sirup as a film under atmospheric pressure on a surface heated to a temperature of about 50° to 120° C.; progressively removing the heated film of sirup from such heated surface in a ripened but ungelled condition; progressively depositing the hot, ripened but ungelled sirup on a surface cooled to a temperature downwards of 20° C.; and progressively removing the cooled film of ungelled sirup from such cooled surface. 105 110
- GEORGE A. RICHTER.
- 40 115
- 45 120
- 50 125
- 55 130
- 60 135
- 65 140
- 70 145
- 75 150